



US008999620B2

(12) **United States Patent**  
**Tanaka et al.**

(10) **Patent No.:** **US 8,999,620 B2**  
(45) **Date of Patent:** **Apr. 7, 2015**

(54) **TONER FOR ELECTROSTATIC LATENT IMAGE DEVELOPMENT**

(71) Applicant: **KYOCERA Document Solutions Inc.**, Osaka-shi (JP)

(72) Inventors: **Takanori Tanaka**, Osaka (JP); **Yukinori Nakayama**, Osaka (JP); **Hiroaki Moriyama**, Osaka (JP); **Takeo Mizobe**, Osaka (JP); **Hiroki Uemura**, Osaka (JP)

(73) Assignee: **KYOCERA Document Solutions Inc.**, Osaka-Shi (JP)

(\*) Notice: Subject to any disclaimer, the term of this patent is extended or adjusted under 35 U.S.C. 154(b) by 0 days.

(21) Appl. No.: **13/954,722**

(22) Filed: **Jul. 30, 2013**

(65) **Prior Publication Data**

US 2014/0038097 A1 Feb. 6, 2014

(30) **Foreign Application Priority Data**

Jul. 31, 2012 (JP) ..... 2012-170576

(51) **Int. Cl.**

**G03G 9/093** (2006.01)  
**G03G 9/08** (2006.01)

(52) **U.S. Cl.**

CPC ..... **G03G 9/09314** (2013.01); **G03G 9/0819** (2013.01); **G03G 9/0827** (2013.01); **G03G 9/09321** (2013.01)

(58) **Field of Classification Search**

USPC ..... 430/110.1, 110.2  
See application file for complete search history.

(56) **References Cited**

U.S. PATENT DOCUMENTS

|                 |   |         |                      |            |
|-----------------|---|---------|----------------------|------------|
| 5,981,129 A     | * | 11/1999 | Akazawa et al. ....  | 430/110.2  |
| 2006/0210899 A1 | * | 9/2006  | Nakazawa et al. .... | 430/106.1  |
| 2007/0042285 A1 | * | 2/2007  | Kitani et al. ....   | 430/110.2  |
| 2008/0166156 A1 | * | 7/2008  | Kawase .....         | 399/222    |
| 2009/0130589 A1 | * | 5/2009  | Udo et al. ....      | 430/137.11 |
| 2009/0297225 A1 | * | 12/2009 | Yamada et al. ....   | 399/252    |
| 2010/0266947 A1 | * | 10/2010 | Maezawa .....        | 430/110.2  |
| 2011/0305984 A1 | * | 12/2011 | Tominaga et al. .... | 430/108.4  |

FOREIGN PATENT DOCUMENTS

|    |               |        |
|----|---------------|--------|
| JP | 2011-070179 A | 4/2011 |
| JP | 2011-133751 A | 7/2011 |
| JP | 2012-137717 A | 7/2012 |

\* cited by examiner

Primary Examiner — Hoa V Le

(74) Attorney, Agent, or Firm — Knobbe Martens Olson & Bear LLP

(57) **ABSTRACT**

A toner for electrostatic latent image development, containing toner particles composed of toner core particle containing at least a binder resin and a shell layer coating the toner core particle. Average circularities  $D_4$  to  $D_7$  of toner particles within predetermined particle diameter ranges are each no less than 0.960, the difference ( $D_{max} - D_{min}$ ) between a maximum value  $D_{max}$  among  $D_4$  to  $D_7$  and a minimum value  $D_{min}$  among  $D_4$  to  $D_7$  is no greater than 0.015. The shell layer is smoothened to a predetermined level. And, cracks in a direction approximately perpendicular to a surface of the toner core particles are observable inside the shell layer when cross-section of the toner particle is observed using a transmission electron microscope.

**4 Claims, 4 Drawing Sheets**



FIG. 1



**FIG. 2**



**FIG. 3**



**FIG. 4**



TONER FOR ELECTROSTATIC LATENT  
IMAGE DEVELOPMENT

## INCORPORATION BY REFERENCE

This application is based upon and claims the benefit of priority from the corresponding Japanese Patent Application No. 2012-170576, filed in the Japan Patent Office on Jul. 31, 2012, the entire contents of which are incorporated herein by reference.

## FIELD

The present disclosure relates to a toner for electrostatic latent image development.

## BACKGROUND

In electrophotography, generally, a surface of a latent image bearing member is charged using a process such as corona discharge followed by exposure using laser to form an electrostatic latent image. The resulting electrostatic latent image is developed by a toner to form a toner image. An image with high quality can be obtained by transferring the resulting toner image on a recording medium. Typically, toner particles (toner base particles) with an average particle diameter of from 5  $\mu\text{m}$  to 10  $\mu\text{m}$ , produced by mixing a binder resin such as a thermoplastic resin with toner components such as a colorant, a charge control agent, a release agent, and a magnetic material and then passing the mixture through the steps of kneading, pulverizing, and classifying, are used for the toner applied to such electrophotography. The above-mentioned method of producing a toner, which includes mixing and kneading the materials in the toner, pulverizing the kneaded material, and classifying the pulverized material, is called a "pulverizing process". In addition, in order to provide flowability or appropriate charging performance to the toner or to facilitate cleaning of the toner from surfaces of photoconductor drums, silica and/or inorganic fine particles such as those of titanium oxide are externally added to the toner base particles.

In regards to such a toner, for the purpose of improving low-temperature fixability, improving high-temperature storage stability, and improving blocking resistance, toner, which includes toner particles of a core-shell structure in which toner core particles using a binder resin of a lower melting point are coated with a shell material consisting of a resin with a glass transition point ( $T_g$ ) higher than that of the binder resin in the toner core particles, have been used heretofore.

As for toner which includes toner particles with such a core-shell structure, a toner which includes toner particles with a core-shell structure, composed of toner core particles containing a polyester resin or a resin where a polyester resin and a vinyl resin are bound and a shell layer consisting of a shell material containing a copolymer between styrene and a (meth)acrylic monomer containing a polyalkylene oxide unit, has been proposed. The toner particles with this core-shell structure are formed by coating a surface of toner core particles with resin fine particles dispersed in an aqueous medium in the presence of an organic solvent such as ethyl acetate.

However, in cases of the toners produced using the pulverizing process, image defects called "void" or "letter scattering" tend to occur in the resulting images. Typically, toner particles in the toners obtained through the pulverizing process exhibit poor flowability because of an irregular shape with a low circularity. When forming images using a toner

containing toner particles with a low circularity, a contact friction coefficient between the toner particles and a surface of latent image bearing member may increase and thus the toner particles may be resistant to be separated from the surface of latent image bearing member. In this case, image defects called "void" may occur in resulting images. Furthermore, in cases where a toner image on a surface of latent image bearing member is transferred on an intermediate transcriptional body such as an intermediate transfer belt and then the toner image on the intermediate transcriptional body is transferred on recording media to thereby form an image, if transfer failure has occurred, image defects called "letter scattering" (phenomenon in which a toner adheres near images such as letters in a condition that the toner is scattered in transferred images) tends to occur in resulting images.

Furthermore, in the shell layers of the toner particles in the toner, since contact sites of the resin fine particles themselves have been dissolved by the organic solvent, there remains almost no void between the resin fine particles and uniform films are formed in a condition that the shape of resin fine particles remains. Therefore, when forming images using the toner, the shell layer may be resistant to break during fixing images on recording media even when a pressure is applied to the toner particles in the toner. In cases where the shell layer cannot be easily broken, it is difficult to appropriately fix the toner on recording media.

In addition to the circumstances described above, in recent years, there is a circumstance that toner particles in toners have been small particle-sized on the ground of growing need for higher image quality. Thin-line reproducibility may be enhanced when images are formed by use of a toner containing toner particles with a smaller particle diameter.

However, the toner containing toner particles with a smaller particle diameter may exhibit lower developing ability. In many cases, the toner containing toner particles with a smaller particle diameter includes an ultrafine powder with a particle diameter of 3  $\mu\text{m}$  or less. When the toner includes the ultrafine powder, the ultrafine powder tends to pollute development sleeve. The ultrafine powder has a strong adhesive force to development sleeve. Therefore, in cases of forming images using a toner containing a large amount of ultrafine powder, the ultrafine powder may stay in development sleeves rather than being supplied to a photoconductor when supplying the toner from the development sleeve to the photoconductor during development. If such a phenomenon is repeated, uneven distribution of the ultrafine powder strongly adhering to development sleeve occurs on the development sleeves (the uneven distribution is called "sleeve adhesion"). If the sleeve adhesion has occurred, developing ability tends to degrade since formation of thin layers of the toner may become insufficient on a peripheral surface of the development sleeves.

## SUMMARY

A toner for electrostatic latent image development of the present disclosure are containing toner particles composed of a toner core particle containing at least a binder resin and a shell layer coating the toner core particle, the shell layer is formed using spherical resin fine particles,

when surfaces of the toner particles are observed with respect to toner particles having a particle diameter from 6  $\mu\text{m}$  to 8  $\mu\text{m}$  using a scanning electron microscope, the structures derived from the spherical resin fine particles are unobservable at the shell layers,

when cross-sections of the toner particles are observed using a transmission electron microscope, cracks are observ-

able inside the shell layers in which the cracks are approximately perpendicular to surfaces of the toner core particles and originate at a phase boundaries of the resin fine particles themselves, and

with respect to average circularities of toner particles in the toner for electrostatic latent image development, an average circularity  $D_4$  of toner particles with a particle diameter of no less than 4  $\mu\text{m}$  and less than 5  $\mu\text{m}$ , an average circularity  $D_5$  of toner particles with a particle diameter of no less than 5  $\mu\text{m}$  and less than 6  $\mu\text{m}$ , an average circularity  $D_6$  of toner particles with a particle diameter of no less than 6  $\mu\text{m}$  and less than 7  $\mu\text{m}$ , and an average circularity  $D_7$  of toner particles with a particle diameter of no less than 7  $\mu\text{m}$  and less than 8  $\mu\text{m}$  are each no less than 0.960, and

the difference ( $D_{\max} - D_{\min}$ ) between a maximum value  $D_{\max}$  among  $D_4$  to  $D_7$  and a minimum value  $D_{\min}$  among  $D_4$  to  $D_7$  is no greater than 0.015.

#### BRIEF DESCRIPTION OF DRAWINGS

FIG. 1 is a view showing a partial cross-section of the toner particle in the toner of the present disclosure;

FIG. 2 is a transmission electron microscope photograph showing a cross-section of the toner particle in the toner of Example 1;

FIG. 3 is a transmission electron microscope photograph showing a cross-section of the toner particle in the toner of Comparative Example 1; and

FIG. 4 is a transmission electron microscope photograph showing a cross-section of the toner particle in the toner of Comparative Example 3.

#### DETAILED DESCRIPTION

The present disclosure is explained in detail with respect to embodiments thereof below; however, the present disclosure is not limited at all to the embodiments and may be carried out with appropriately making a change within the purpose of the present disclosure. In addition, explanation may be occasionally omitted with respect to duplicated matters; this does not however limit the gist of the present disclosure.

Hereinafter, in the case of the toner of the present disclosure, the structure of the toner particles and materials of the toner particles are explained.

##### Structure of Toner Particles

In the toner particles in the toner of the present disclosure, the entire surfaces of the toner core particles are coated with the shell layers. Surface conditions of the toner particles coated with the shell layers can be confirmed using a scanning electron microscope (SEM). Smoothened levels of the shell layers and inner structures of the shell layers of the toner particles can be confirmed by observing cross-sections of the toner particles using a transmission electron microscope (TEM). FIG. 1 shows a schematic cross-sectional view, which is observed using a TEM, of toner particles in the toner in accordance with one preferable embodiment of the present disclosure.

As shown in FIG. 1, in the toner particle 101 in the toner for electrostatic latent image development, the shell layer 103 covers the entire surface of the toner core particle 102. The shell layer is formed by smoothening an outer surface of a layer of resin fine particles, which has been formed by adhering the resin fine particles onto toner core particle, using an external force.

The thickness of the shell layer 103 is preferably from 0.03  $\mu\text{m}$  to 1  $\mu\text{m}$ , more preferably from 0.04  $\mu\text{m}$  to 0.7  $\mu\text{m}$ , particularly preferably from 0.045  $\mu\text{m}$  to 0.5  $\mu\text{m}$ , and most pref-

erably from 0.045  $\mu\text{m}$  to 0.3  $\mu\text{m}$ . When the shell layer has convex parts, the shell layer may be uneven in its thickness, as described later. In cases where the shell layer is uneven in its thickness like this, the thickness at the thickest part of the shell layer is defined as "the thickness of the shell layer" in claims and specification of the present application.

When forming images using a toner which includes toner particles with an excessively thick shell layer, the shell layers are resistant to break even if a pressure is applied to the toner particles during fixing the toner to recording media. In this case, it is difficult to fix the toner in a low-temperature region since softening or melting of binder resins and/or release agents in toner core particles does not promptly proceed. On the other hand, an excessively thin shell layer leads to a lower strength. When the strength of the shell layer is low, the shell layer may be broken due to a shock occurring during a state like transportation. In cases where toners are stored at high temperatures, toner particles with a shell layer broken at least partially tend to agglomerate. The reason is that components such as a release agent tend to exude onto a surface of the toner particle through the site where the shell layer has been broken.

The thickness of the shell layer 103 may be measured by analyzing a TEM image of a cross-section of the toner particle 101 using commercially available image analysis software. Software such as WINROOF (by MITANI Co.) may be used as the commercially available image analysis software.

As shown in FIG. 1, preferably, the shell layer 103 has convex parts 105 between two cracks 104 on the phase boundary between the toner core particle 102 and the shell layer 103. By having such convex parts 105 in the shell layer 103, the contact area between the toner core particle 102 and the shell layer 103 is larger than that of the case where the shell layer has no convex part 105. Therefore, when the shell layer 103 has the convex parts 105, the toner core particle 102 and the shell layer 103 appropriately adhere, and thus the shell layer 103 is unlikely to peel from the toner core particle 102. Therefore, by having the convex parts 105 in the shell layer 103, a toner with excellent heat-resistant storage stability can be obtained.

More specifically, the shell layer formed using resin fine particles is formed by a method including:  
 I) a step of making spherical resin fine particles adhere to the surface of toner core particle so as to not overlap in a direction perpendicular to the surface of toner core particle and forming a layer of the resin fine particles that covers the entire surface of the toner core particle, and  
 II) a step of forming a shell layer by applying an external force to the outer surface of the layer of the resin fine particles and deforming the resin fine particles in the layer of the resin fine particles to thereby smoothen the outer surface of the layer of the resin fine particles.

The smoothened level of the shell layer may be such a level that the structures derived from the spherical resin fine particles used for forming the shell layer cannot be observed at the outer surfaces of the shell layers of toner particles having a particle diameter from 6  $\mu\text{m}$  to 8  $\mu\text{m}$  when observing the surfaces of the toner particles using a scanning electron microscope. When the toner particles having a particle diameter from 6  $\mu\text{m}$  to 8  $\mu\text{m}$  represent such a condition in the shell layer, in almost all the toner particles in the toner, the shell layers have been formed such that the surface of the toner core particles are not exposed. In a case that the condition of outer surface of the shell layer is confirmed using the scanning electron microscope, the particle diameter of a toner particle is an equivalent circle diameter calculated from a projected area of the toner particles on an electron microscope image.

In the preferable embodiment of the shell layer shown in FIG. 1, the entire surface of the toner core particle 102 is coated by the shell layer 103. Since the shell layer 103 covers the entire surface of the toner core particle 102 such that its outer surface is smooth, components such as a release agent are unlikely to exude onto a surface of the toner particle 101 during storage of the toner particle 101 at high temperatures.

There are voids (cracks) 104 inside the shell layer 103. Therefore, when a pressure is applied to the toner for fixing the toner particles on recording media, the shell layer is likely to break from a crack as an origin. When the shell layer is promptly broken, then softening or melting of components such as a binder resin and a release agent in the toner core particles 102 promptly proceeds, thus the toner can be fixed on recording media at a temperature lower than heretofore.

In the toner of the present disclosure, with respect to average circularities of toner particles in the toner, an average circularity  $D_4$  of toner particles with a particle diameter of no less than 4  $\mu\text{m}$  and less than 5  $\mu\text{m}$ , an average circularity  $D_5$  of toner particles with a particle diameter of no less than 5  $\mu\text{m}$  and less than 6  $\mu\text{m}$ , an average circularity  $D_6$  of toner particles with a particle diameter of no less than 6  $\mu\text{m}$  and less than 7  $\mu\text{m}$ , and an average circularity  $D_7$  of toner particles with a particle diameter of no less than 7  $\mu\text{m}$  and less than 8  $\mu\text{m}$  are each no less than 0.960; and the difference ( $D_{\max} - D_{\min}$ ) between a maximum value  $D_{\max}$  among  $D_4$  to  $D_7$ , and a minimum value  $D_{\min}$  among  $D_4$  to  $D_7$  is no greater than 0.015.

Toners not satisfying the above-noted conditions in terms of  $D_4$  to  $D_7$  thereof may include many toner particles with a less round shape in the toners. In this case, the contact friction coefficient between the toner particles and a surface of latent image bearing member may increase and thus the toner particles are resistant to be separated from the surface of latent image bearing member when toner images are transferred from the latent image bearing member to recording media. In such a case, transfer void arises in resulting images and image defects occur in the resulting images.

In regards to the toner of the present disclosure, if ( $D_{\max} - D_{\min}$ ) is greater than 0.015 in the toner, variation occurs in the contact friction coefficient between the toner particles and latent image bearing member since variation in the circularity distribution of the toner particles is larger than desired. Therefore, the toner particles become resistant to be uniformly separated from the surface of latent image bearing member when toner images are transferred from the latent image bearing member to recording media. In such a case, image defects due to the occurrence of transfer void may occur in resulting images.

In cases where ( $D_{\max} - D_{\min}$ ) is greater than 0.015, variation in charged amounts of toner particles becomes larger than desired due to the variation in circularities of toner particles and thus the charged amount distribution of the toner becomes broader than desired. When the charged amount distribution of the toner has become broader than desired, agglomeration of charged particles themselves in the toner tends to occur on developing sleeve. In this case, it is difficult to form a uniform toner layer on the developing sleeve and thus an image defect (unevenness in sleeve layers) tends to occur in resulting images.

The average circularities  $D_4$  to  $D_7$  can be measured in accordance with the method below.

#### Method of Calculating Circularity

Using a Flow Particle Image Analyzer (FPIA-3000, by Sysmex Co.), an average circularity of toner particles in the toner of the present disclosure is calculated. Under an environment of 23° C. and 60% RH, a circumferential length ( $L_0$ ) of a circle having a projected area the same as that of a particle

image and a peripheral length (L) of a particle projected image are measured for all of toner particles to be measured. Circularity is calculated in accordance with the formula below. Using the data of toner particles, among all toner particles to be measured, having an equivalent circle diameter within a range of no less than 4.0  $\mu\text{m}$  and less than 8.0  $\mu\text{m}$ , average circularities  $D_4$ ,  $D_5$ ,  $D_6$ , and  $D_7$  described below are calculated.

#### (Formula to Calculate Average Circularity)

$$10 \quad \text{Average circularity} = L_0/L$$

(Average Circularity  $D_4$  of Toner Particles with Particle Diameter of No Less than 4  $\mu\text{m}$  and Less than 5  $\mu\text{m}$ )

The sum of circularities of toner particles to be measured 15 with an equivalent circle diameter of no less than 4  $\mu\text{m}$  and less than 5  $\mu\text{m}$  is divided by the total particle number of toner particles to be measured with an equivalent circle diameter of no less than 4  $\mu\text{m}$  and less than 5  $\mu\text{m}$ , and the resulting value is defined as the average circularity  $D_4$ .

(Average Circularity  $D_5$  of Toner Particles with Particle Diameter of No Less than 5  $\mu\text{m}$  and Less than 6  $\mu\text{m}$ )

The sum of circularities of toner particles to be measured with an equivalent circle diameter of no less than 5  $\mu\text{m}$  and less than 6  $\mu\text{m}$  is divided by the total particle number of toner 25 particles to be measured with an equivalent circle diameter of no less than 5  $\mu\text{m}$  and less than 6  $\mu\text{m}$ , and the resulting value is defined as the average circularity  $D_5$ .

(Average Circularity  $D_6$  of Toner Particles with Particle Diameter of No Less than 6  $\mu\text{m}$  and Less than 7  $\mu\text{m}$ )

The sum of circularities of toner particles to be measured 30 with an equivalent circle diameter of no less than 6  $\mu\text{m}$  and less than 7  $\mu\text{m}$  is divided by the total particle number of toner particles to be measured with an equivalent circle diameter of no less than 6  $\mu\text{m}$  and less than 7  $\mu\text{m}$ , and the resulting value is defined as the average circularity  $D_6$ .

(Average Circularity  $D_7$  of Toner Particles with Particle Diameter of No Less than 7  $\mu\text{m}$  and Less than 8  $\mu\text{m}$ )

The sum of circularities of toner particles to be measured 35 with an equivalent circle diameter of no less than 7  $\mu\text{m}$  and less than 8  $\mu\text{m}$  is divided by the total particle number of toner particles to be measured with an equivalent circle diameter of no less than 7  $\mu\text{m}$  and less than 8  $\mu\text{m}$ , and the resulting value is defined as the average circularity  $D_7$ .

The values of  $D_4$  to  $D_7$  and ( $D_{\max} - D_{\min}$ ) can be adjusted by 40 controlling an amount of resin fine particles used when forming a shell layer and/or a circularity of toner core particles, as described below. By increasing an amount of resin fine particles used when producing the toner particles, each value of  $D_4$  to  $D_7$  can be increased and the value of ( $D_{\max} - D_{\min}$ ) can be decreased. By decreasing an amount of resin fine particles used when producing the toner, each value of  $D_4$  to  $D_7$  can be decreased and the value of ( $D_{\max} - D_{\min}$ ) can be increased.

#### Material of Toner Particles

The toner particles in the toner are composed of toner core 55 particles containing at least a binder resin and the shell layers coating the entire surfaces of the toner core particles. The toner core particles may contain components such as a release agent, a charge control agent, a colorant, and a magnetic powder in the binder resin as required. The surfaces of the toner particles may be treated using an external additive as required. The toner may be mixed with a desired carrier and used as a two-component developer.

Hereinafter, the binder resin, the release agent, the charge 60 control agent, the colorant, the magnetic powder, the resin fine particles for forming the shell layer, and external additives, which are essential or optional components to configure the toner particles, the carrier which is used in a case of using

the toner as a two component developer, and a method of producing the toner particles are explained in order.

#### Binder Resin

The toner core particles contain a binder resin. The binder resin in the toner core particles is not particularly limited as long as it is a resin used heretofore as a binder resin for toners. Specific examples of the binder resin are thermoplastic resins such as polystyrene resins, acrylic resins, styrene-acrylic resins, polyethylene resins, polypropylene resins, vinyl chloride resins, polyester resins, polyamide resins, polyurethane resins, polyvinyl alcohol resins, vinyl ether resins, N-vinyl resins, and styrene-butadiene resins. Among these resins, polystyrene resins and polyester resins are preferable from the viewpoints of dispersibility of colorants in the binder resin, charging ability of the toner, and fixability on paper. Hereinafter, the polystyrene resin and the polyester resin are explained.

The polystyrene resin may be a styrene homopolymer or a copolymer between styrene and other copolymerization monomers copolymerizable with styrene. Specific examples of the other copolymerization monomers copolymerizable with styrene are p-chlorostyrene; vinylnaphthalene; ethylenically unsaturated monoolefins such as ethylene, propylene, butylene, and isobutylene; halogenated vinyls such as vinyl chloride, vinyl bromide, and vinyl fluoride; vinyl esters such as vinyl acetate, vinyl propionate, vinyl benzoate, and vinyl butyrate; (meth)acrylic acid esters such as methyl acrylate, ethyl acrylate, n-butyl acrylate, isobutyl acrylate, dodecyl acrylate, n-octyl acrylate, 2-chloroethyl acrylate, phenyl acrylate,  $\alpha$ -methyl chloroacrylate, methyl methacrylate, ethyl methacrylate, and butyl methacrylate; other acrylic acid derivatives such as acrylonitrile, methacrylonitrile, and acrylamide; vinyl ethers such as vinyl methyl ether and vinyl isobutyl ether; vinyl ketones such as vinyl methyl ketone, vinyl ethyl ketone, and methyl isopropenyl ketone; and N-vinyl compounds such as N-vinyl pyrrole, N-vinyl carbazole, N-vinyl indole, and N-vinyl pyrrolidene. These copolymerization monomers may be copolymerized with styrene monomer in a combination of two or more.

The polyester resin may be those obtained through condensation polymerization or co-condensation polymerization of bivalent, trivalent or higher-valent alcohol components and bivalent, trivalent or higher-valent carboxylic acid components. The components used for synthesizing the polyester resin may be exemplified by the alcohol components and the carboxylic acid components below.

Specific examples of the divalent, trivalent or higher-valent alcohols may be exemplified by diols such as ethylene glycol, diethylene glycol, triethylene glycol, 1,2-propylene glycol, 1,3-propylene glycol, 1,4-butanediol, neopentyl glycol, 1,4-butanediol, 1,5-pentanediol, 1,6-hexanediol, 1,4-cyclohexane dimethanol, dipropylene glycol, polyethylene glycol, polypropylene glycol, and polytetramethylene glycol; bisphenols such as bisphenol A, hydrogenated bisphenol A, polyoxyethylenated bisphenol A, and polyoxypropylenated bisphenol A; and trivalent or higher-valent alcohols such as sorbitol, 1,2,3,6-hexanetetrol, 1,4-sorbitane, pentaerythritol, dipentaerythritol, tripentaerythritol, 1,2,4-butanetriol, 1,2,5-pentanetriol, glycerol, diglycerol, 2-methylpropanetriol, 2-methyl-1,2,4-butanetriol, trimethylolethane, trimethylolpropane, and 1,3,5-trihydroxymethylbenzene.

Specific examples of the divalent, trivalent or higher-valent carboxylic acids include divalent carboxylic acids such as maleic acid, fumaric acid, citraconic acid, itaconic acid, glutaconic acid, phthalic acid, isophthalic acid, terephthalic acid, cyclohexane dicarboxylic acid, succinic acid, adipic acid, sebacic acid, azealic acid, malonic acid, or alkyl or

alkenyl succinic acids including n-butyl succinic acid, n-butylsuccinic acid, isobutylsuccinic acid, isobutensylsuccinic acid, n-octylsuccinic acid, n-octenylsuccinic acid, n-dodecylsuccinic acid, n-dodecenylsuccinic acid, isododecylsuccinic acid, isododecylsuccinic acid; and trivalent or higher-valent carboxylic acids such as 1,2,4-benzene tricarboxylic acid (trimellitic acid), 1,2,5-benzene tricarboxylic acid, 2,5,7-naphthalene tricarboxylic acid, 1,2,4-naphthalene tricarboxylic acid, 1,2,4-butane tricarboxylic acid, 1,2,5-hexane tricarboxylic acid, 1,3-dicarboxyl-2-methyl-2-methylene carboxypropane, 1,2,4-cyclohexane tricarboxylic acid, tetra(methylenecarboxyl)methane, 1,2,7,8-octanetetracarboxylic acid, pyromellitic acid, and Enpol trimer. These divalent, trivalent or higher-valent carboxylic acids may be used as ester-forming derivatives such as an acid halide, an acid anhydride, and a lower alkyl ester. Here, the term "lower alkyl" means an alkyl group of from 1 to 6 carbon atoms.

When the binder resin is a polyester resin, the softening point of the polyester resin is preferably from 70° C. to 130° C. and more preferably 80° C. to 120° C.

In a case that the toner is used as a magnetic one-component developer, preferably, a resin having at least one functional group selected from the group consisting of hydroxyl group, carboxyl group, amino group, and epoxy group (glycidyl group) in its molecule is used as the binder resin. By use of the binder resin having these functional groups in its molecule, dispersibility of components such as a magnetic powder and a charge control agent in the binder resin can be improved. Presence or absence of these functional groups can be confirmed using a Fourier transform infrared spectrophotometer (FT-IR). The amount of these functional groups in the resins can be measured using conventional processes such as titration.

A thermoplastic resin is preferable as the binder resin since a toner with an appropriate fixability to paper may be easily obtained; here, the thermoplastic resin may be used together with a cross-linking agent and/or a thermosetting resin. By adding the cross-linking agent and/or the thermosetting resin and introducing a partial cross-linked structure into the binder resin, heat-resistant storage stability and durability of the toner may be improved without degrading the fixability of the toner. When a thermosetting resin is used together with the thermoplastic resin, the amount of cross-linked part (gel amount) in the binder resin extracted using a Soxhlet extractor is preferably no greater than 10% by mass and more preferably from 0.1% to 10% by mass based on the mass of the binder resin.

The thermosetting resin usable together with the thermoplastic resin is preferably epoxy resins and cyanate resins. Specific examples of preferable thermosetting resins are bisphenol A-type epoxy resins, hydrogenated bisphenol A-type epoxy resins, novolak-type epoxy resins, polyalkylene ether-type epoxy resins, cyclic aliphatic-type epoxy resins, and cyanate resins. These thermosetting resins may be used in a combination of two or more.

The glass transition point (Tg) of the binder resin is preferably from 40° C. to 70° C. A toner which includes toner particles obtained using a binder resin with an excessively high glass transition point tends to exhibit poor low-temperature fixability. A toner which includes toner particles obtained using a binder resin with an excessively low glass transition point tends to exhibit poor heat-resistant storage stability.

The glass transition point of the binder resin can be determined from a changing point of specific heat of the binder resin using a differential scanning calorimeter (DSC). More specifically, the glass transition point of the binder resin can be determined by measuring an endothermic curve using a

differential scanning calorimeter (DSC-6200, by Seiko Instruments Inc.) as a measuring device.

10 mg of a sample to be measured is loaded into an aluminum pan and an empty aluminum pan is used as a reference. The glass transition point of the binder resin can be determined from an endothermic curve of the binder resin that is obtained by measuring under a measuring temperature range of from 25° C. to 200° C., a temperature-increase rate of 10° C./min, and normal temperature and normal humidity.

The mass average molecular mass (Mw) of the binder resin is preferably from 20,000 to 300,000 and more preferably from 30,000 to 200,000. The mass average molecular mass (Mw) of the binder resin can be determined using gel permeation chromatography (GPC) based on a calibration curve previously prepared using standard polystyrene resins.

When the binder resin is a polystyrene resin, preferably, the binder resin has a peak in a region of lower molecular masses and a peak in a region of higher molecular masses respectively in terms of molecular mass distribution measured by a means such as gel permeation chromatography. Specifically, the peak of molecular mass in a region of lower molecular masses is preferably within a range from 3,000 to 20,000 and the peak of molecular mass in a region of higher molecular masses is preferably within a range from 300,000 to 1,500,000. It is preferred for the polystyrene resin having such a molecular mass distribution that a ratio (Mw/Mn) of a mass average molecular mass (Mw) to a number average molecular mass (Mn) is at least 10. By use of the binder resin having a peak respectively in a region of lower molecular masses and a region of higher molecular masses, a toner excellent in low-temperature fixability and allowing to suppress high-temperature offset can be obtained.

#### Release Agent

The toner core particles preferably contain a release agent in order to improve fixability and offset resistance. The release agent is preferably a wax. Examples of the wax include carnauba wax, synthetic ester wax, polyethylene wax, polypropylene wax, fluorine resin wax, Fischer-Tropsch wax, paraffin wax, montan wax, and rice wax. These release agents may be used in a combination of two or more. The occurrence of offset and/or image smearing (smear around images occurring upon rubbing the images) may be more effectively suppressed by adding the release agent to the toner.

In cases where a polyester resin is used as the binder resin, preferably, at least one release agent selected from the group consisting of carnauba wax, synthetic ester wax, and polyethylene wax is used from the viewpoint of compatibility between the binder resin and the release agent. In cases where a polystyrene resin is used as the binder resin, preferably, Fischer-Tropsch wax and/or paraffin wax is used similarly from the viewpoint of compatibility between the binder resin and the release agent.

The Fischer-Tropsch wax is a linear hydrocarbon compound, produced by Fischer-Tropsch reaction of a catalytic hydrogenation reaction of carbon monoxide, which has a small content of iso-structural molecules and/or side chains.

Among Fischer-Tropsch waxes, those having a mass average molecular mass of 1,000 or higher and exhibiting a bottom temperature in endothermic peaks observed by DSC measurement within a range from 100° C. to 120° C. are more preferable. Such a Fischer-Tropsch wax may be exemplified by Sasol Wax C1 (bottom temperature in endothermic peaks: 106.5° C.), Sasol Wax C105 (bottom temperature in endothermic peaks: 102.1° C.), and Sasol Wax SPRAY (bottom temperature in endothermic peaks: 102.1° C.) which are available from Sasol Wax GmbH.

The amount of the release agent used is preferably from 1% to 10% by mass based on the total mass of the toner core particles. When using a toner which includes toner particles in which the content of the release agent is excessively small, the desired effect for suppressing the occurrence of offset or image smearing in the resulting images may not be obtained. A toner which includes toner particles with an excessively large content of the release agent may degrade the heat-resistant storage stability of the toner since toner particles tend to agglomerate.

#### Charge Control Agent

Preferably, the toner core particles contain a charge control agent for the purpose of improving a charged level or a charge-increasing property, which is an indicator of chargeability to a predetermined charged level within a short time, of the toner particles, to thereby obtain a toner excellent in durability and stability. When the toner particles in the toner are positively charged to develop, a positively chargeable charge control agent is used; and when the toner particles in the toner are negatively charged to develop, a negatively chargeable charge control agent is used.

The charge control agent may be appropriately selected from conventional charge control agents used for toners heretofore. Specific examples of the positively chargeable charge control agent are azine compounds such as pyridazine, pyrimidine, pyrazine, ortho-oxazine, meta-oxazine, para-oxazine, ortho-thiazine, meta-thiazine, para-thiazine, 1,2,3-triazine, 1,2,4-triazine, 1,3,5-triazine, 1,2,4-oxadiazine, 1,3,4-oxadiazine, 1,2,6-oxadiazine, 1,3,4-thiadiazine, 1,3,5-thiadiazine, 1,2,3,4-tetrazine, 1,2,4,5-tetrazine, 1,2,3,5-tetrazine, 1,2,4,6-oxatriazine, 1,3,4,5-oxatriazine, phthalazine, quinazoline, and quinoxaline; direct dyes consisting of azine compounds such as azine FastRed FC, azine FastRed 12BK, azine Violet BO, azine Brown 3G, azine Light Brown GR, azine Dark Green BH/C, azine Deep Black EW, and azine Deep Black 3RL; nigrosine compounds such as nigrosine, nigrosine salts, and nigrosine derivatives; acid dyes consisting of nigrosine compounds such as nigrosine BK, nigrosine NB, and nigrosine Z; metal salts of naphthenic acid or higher fatty acid; alkoxylated amines; alkylamides; quaternary ammonium salts such as benzylmethylhexyldecyl ammonium, and decyltrimethylammonium chloride. Among these positively chargeable charge control agents, nigrosine compounds are particularly preferable since a more rapid charge-increasing property may be obtained. These positively chargeable charge control agents may be used in a combination of two or more.

Resins having a quaternary ammonium salt, a carboxylic acid salt, or a carboxyl group as a functional group may also be used as the positively chargeable charge control agent. More specifically, styrene resins having a quaternary ammonium salt, acrylic resins having a quaternary ammonium salt, styrene-acrylic resins having a quaternary ammonium salt, polyester resins having a quaternary ammonium salt, styrene resins having a carboxylic acid salt, acrylic resins having a carboxylic acid salt, styrene-acrylic resins having a carboxylic acid salt, polyester resins having a carboxylic acid salt, styrene resins having a carboxylic group, acrylic resins having a carboxylic group, styrene-acrylic resins having a carboxylic group, and polyester resins having a carboxylic group may be exemplified. These resins may be an oligomer or a polymer.

Among the resins usable as the positively chargeable charge control agent, styrene-acrylic resins having a quaternary ammonium salt as a functional group are more preferable since the charged amount may be easily controlled within a desired range. In regards to the styrene-acrylic resins

## 11

having a quaternary ammonium salt as a functional group, preferable specific examples of acrylic comonomers copolymerized with a styrene unit are (meth)acrylic acid alkyl esters such as methyl acrylate, ethyl acrylate, n-propyl acrylate, iso-propyl acrylate, n-butyl acrylate, iso-butyl acrylate, 2-ethylhexyl acrylate, methyl methacrylate, ethyl methacrylate, n-butyl methacrylate, and iso-butyl methacrylate.

The units derived from dialkylamino alkyl(meth)acrylates, dialkyl(meth)acrylamides, or dialkylamino alkyl(meth)acrylamides through a quaternizing step may be used as the quaternary ammonium salt. Specific examples of the dialkylamino alkyl(meth)acrylate are dimethylamino ethyl(meth)acrylate, diethylamino ethyl(meth)acrylate, dipropylamino ethyl(meth)acrylate, and dibutylamino ethyl(meth)acrylate; a specific example of the dialkyl(meth)acrylamide is dimethyl methacrylamide; and a specific example of the dialkylamino alkyl(meth)acrylamide is dimethylamino propylmethacrylamide. Additionally, hydroxyl group-containing polymerizable monomers such as hydroxy ethyl(meth)acrylate, hydroxy propyl(meth)acrylate, 2-hydroxy butyl(meth)acrylate, and N-methylol(meth)acrylamide may also be used in combination at the time of polymerization.

Specific examples of the negatively chargeable charge control agent are organic metal complexes, chelate compounds, monoazo metal complexes, acetylacetone metal complexes, aromatic hydroxycarboxylic acids, metal complexes of aromatic dicarboxylic acids, aromatic monocarboxylic acids, aromatic polycarboxylic acids, and metal salts, anhydrides, or esters thereof, and phenol derivatives such as bisphenol. Among these, organic metal complexes and chelate compounds are preferable. Among organic metal complexes and chelate compounds, acetylacetone metal complexes such as aluminum acetylacetone and iron(II) acetylacetone and salicylic acid metal complexes or salicylic acid metal salts such as 3,5-di-tert-butylsalicylic acid chromium are more preferable, and salicylic acid metal complexes or salicylic acid metal salts are particularly preferable. These negatively chargeable charge control agents may be used in a combination of two or more.

The amount of the positively or negatively chargeable charge control agent used is preferably from 0.1% to 10% by mass based on the total mass of the toner core particles. In cases of using a toner, which includes toner particles where the content of the charge control agent is excessively small, image density of the resulting images may be lower than a desired value or it may be difficult to maintain image density of the resulting images for a long period since it is difficult to stably charge the toner particles in a predetermined polarity. Moreover, in cases where the content of the charge control agent is excessively small in the toner particles, since it is difficult to uniformly disperse the charge control agent in the binder resin, fogging tends to occur in the resulting images or smear caused by toner components tends to occur in latent image bearing members. In cases of using a toner, which includes toner particles where the content of the charge control agent is excessively large, smear caused by toner components tends to occur in latent image bearing members or image defects due to an inferior charge under high temperature and high humidity caused by degradation of environmental resistance tend to occur in the resulting images.

## Colorant

The toner core particles may contain a colorant as required. Conventional pigments or dyes may be used as the colorant depending on the color of the toner. Specific examples of the colorant are black pigments such as carbon black, acetylene black, lamp black, and aniline black; yellow pigments such as chrome yellow, zinc yellow, cadmium yellow, yellow iron

## 12

oxide, mineral fast yellow, nickel titanium yellow, nables yellow, naphthol yellow S, hanza yellow G, hansa yellow 10G, benzidine yellow G, benzidine yellow GR, quinoline yellow lake, permanent yellow NCG, turtrazine lake, monoazo yellow, and diazo yellow; orange pigments such as red chrome yellow, molybdenum orange, permanent orange GTR, pyrazolone orange, balkan orange, and indanthrene brilliant orange GK; red pigments such as iron oxide red, cadmium red, minium, cadmium mercury sulfate, permanent red 4R, lisol red, pyrazolone red, watching red calcium salt, lake red D, brilliant carmine 6B, eosine lake, rhodamine lake B, alizarin lake, brilliant carmine 3B, and monoazo red; violet pigments such as manganese violet, fast violet B, and methyl violet lake; blue pigments such as pigment blue 27, cobalt blue, alkali blue lake, Victoria blue partially chlorinated product, fast sky blue, indanthrene blue BC, and phthalocyanine blue; green pigments such as chrome green, chromium oxide, pigment green B, malachite green lake, and final yellow green G; white pigments such as zinc white, titanium dioxide, antimony white, and zinc sulfate; and extender pigments such as barite powder, barium carbonate, clay, silica, white carbon, talc, and alumina white. These colorants may be used in a combination of two or more for the purpose of tailoring the toner to a desired hue.

The amount of the colorant used is preferably from 1% to 10% by mass and more preferably from 2% to 7% by mass based on the total mass of the toner core particles.

The colorant may also be used as a master batch where the colorant has been previously dispersed in a resin material such as a thermoplastic resin. When using the colorant as a master batch, the resin in the master batch is preferably of the same type as that of the binder resin.

## Magnetic Powder

The toner core particles may contain a magnetic powder as required. The toner, which includes toner particles is composed of toner core particles containing the magnetic powder in the binder resin and a shell layer coating the toner core particles, may be used as a magnetic one-component developer. The magnetic powder may be exemplified by iron oxides such as ferrite and magnetite, ferromagnetic metals such as those of cobalt and nickel, alloys of iron and/or ferromagnetic metals, compounds of iron and/or ferromagnetic metals, ferromagnetic alloys via ferromagnetizing treatment like heat-treatment, and chromium dioxide.

The particle diameter of the magnetic powder is preferably from 0.1  $\mu\text{m}$  to 1.0  $\mu\text{m}$  and more preferably from 0.1  $\mu\text{m}$  to 0.5  $\mu\text{m}$ . When preparing the toner core particles using the magnetic powder with a particle diameter within this range, the magnetic powder may be easily dispersed into the binder resin.

In order to improve dispersibility into the binder resin, the magnetic powder surface-treated with a surface treatment agent such as a titanium coupling agent and/or a silane coupling agent may also be used.

The amount of the magnetic powder used is preferably from 35% to 65% by mass and more preferably from 35% to 55% by mass based on the total mass of the toner core particles. In cases of using a toner, which includes toner particles composed of toner core particles where the content of the magnetic powder is excessively large and a shell layer coating the toner core particles, it may be difficult to form images with an intended image density when forming images continuously for a long period or fixability may be extremely deteriorated. In cases of using a toner, which includes toner particles composed of toner core particles where the content of the magnetic powder is excessively small and a shell layer coating the toner core particles, fogging tends to occur in the

60  
65

resulting images or image density of resulting images may be decreased when printing images for a long period.

### The resin fine par-

The resin fine particles for forming the shell layer are not particularly limited as long as they can coat the toner core particles. The resin fine particles for forming the shell layer are preferably a polymer of a monomer having an unsaturated bond since a shell layer with a predetermined structure may be easily formed. Preferably, the resin fine particles contain a resin that can be synthesized by a soap-free emulsion polymerization. The reason is that producing the resin fine particles by the soap-free emulsion polymerization allows the preparation of resin fine particles where their particle diameters are uniform and no or almost no surfactant is included.

The monomer having an unsaturated bond is not particularly limited as long as it is a monomer from which a resin having sufficient physical properties as the shell layer can be synthesized. The monomer having an unsaturated bond is preferably a vinyl monomer. The vinyl group in the vinyl monomer may be substituted at  $\alpha$ -site thereof with an alkyl group. The vinyl group in the vinyl monomer may also be substituted with a halogen atom. The alkyl group, which the vinyl group may have, is preferably an alkyl group of from 1 to 6 carbon atoms, more preferably methyl or ethyl group, and particularly preferably methyl group. The halogen atom, which the vinyl group may have, is preferably chlorine or bromine atom and more preferably chlorine atom.

The vinyl monomer may also have a nitrogen-containing polar functional group or a fluorine-substituted hydrocarbon group. In a case of using a vinyl monomer having a nitrogen-containing polar functional group when producing a resin, positively chargeable property can be imparted to the resulting resin. In a case of using a vinyl monomer having a fluorine-substituted hydrocarbon group when producing a resin, negatively chargeable property can be imparted to the resulting resin. In a case of using the positively chargeable resin or the negatively chargeable resin as the material of the shell layer, a toner chargeable to an intended charged amount may be obtained even when no charge control agent is compounded in the toner core particles or the amount of the charge control agent compounded in the toner core particles is reduced.

Among vinyl monomers, specific examples of the monomer having no nitrogen-containing polar functional group or fluorine-substituted hydrocarbon group are styrenes such as styrene, o-methylstyrene, m-methylstyrene, p-methylstyrene, p-ethylstyrene, 2,4-dimethylstyrene, p-n-butylstyrene, p-tert-butylstyrene, p-n-hexylstyrene, p-n-octylstyrene, p-n-nonylstyrene, p-n-decylstyrene, p-n-dodecylstyrene, p-methoxystyrene, p-ethoxystyrene, p-phenylstyrene, p-chlorostyrene, and 3,4-dichlorostyrene; ethylenically unsaturated monoolefins such as ethylene, propylene, butylene, and isobutylene; halogenated vinyls such as vinyl chloride, vinylidene chloride, vinyl bromide, and vinyl fluoride; vinyl esters such as vinyl acetate, vinyl propionate, vinyl benzoate, and vinyl butyrate; (meth)acrylic acid esters such as methyl (meth)acrylate, ethyl (meth)acrylate, n-butyl (meth)acrylate, isobutyl(meth)acrylate, propyl(meth)acrylate, n-octyl(meth)acrylate, dodecyl(meth)acrylate, 2-ethylhexyl(meth)acrylate, stearyl(meth)acrylate, 2-chloroethyl(meth)acrylate, phenyl(meth)acrylate, and methyl  $\alpha$ -chloroacrylate; (meth) acrylic acid derivatives such as acrylonitrile; vinyl ethers such as vinyl methyl ether, vinyl ethyl ether, and vinyl isobutyl ether; vinyl ketones such as vinyl methyl ketone, vinyl hexyl ketone, and methyl isopropenyl ketone; and vinyl naphtha-

lines. Among these, styrenes are preferable and styrene is more preferable. These monomers may be used in a combination of two or more.

Examples of the vinyl monomer having a nitrogen-containing polar functional group are N-vinyl compounds, amino(meth)acrylic monomers, methacrylonitrile, and (meth)acrylic amide. Specific examples of the N-vinyl compounds are N-vinyl pyrrole, N-vinyl carbazole, N-vinyl indole, and N-vinyl pyrrolidone. Preferable examples of the amino(meth)acrylic monomer are the compounds represented by the formula below:



(in the formula,  $R^1$  represents hydrogen or a methyl group;  $R^2$  and  $R^3$  respectively represent a hydrogen atom or an alkyl group of from 1 to 20 carbon atoms;  $X$  represents  $-\text{O}-$ ,  $-\text{O}-\text{Q}-$ , or  $-\text{NH}$ ; and  $Q$  represents an alkylene group of from 1 to 10 carbon atoms, a phenylene group, or a combination of these groups).

In the above-mentioned formula, specific examples of  $R^2$  and  $R^3$  are methyl group, ethyl group, n-propyl group, iso-propyl group, n-butyl group, iso-butyl group, sec-butyl group, tert-butyl group, n-pentyl group, iso-pentyl group, tert-pentyl group, n-hexyl group, n-heptyl group, n-octyl group, 2-ethylhexyl group, n-nonyl group, n-decyl group, n-undecyl group, n-dodecyl group (lauryl group), n-tridecyl group, n-tetradecyl group, n-pentadecyl group, n-hexadecyl group, n-heptadecyl group, n-octadecyl group (stearyl group), n-nonadecyl group, and n-icosyl group.

In the above-mentioned formula, specific examples of Q are methylene group, 1,2-ethanediyl group, 1,1-ethylene group, propane-1,3-diyl group, propane-2,2-diyl group, propane-1,1-diyl group, propane-1,2-diyl group, butane-1,4-diyl group, pentane-1,5-diyl group, hexane-1,6-diyl group, heptane-1,7-diyl group, octane-1,8-diyl group, nonane-1,9-diyl group, decane-1,10-diyl group, p-phenylene group, m-phenylene group, o-phenylene group, and a divalent group without hydrogen at 4-site of phenyl group in a benzyl group.

diethylaminophenyl)methyl (meth)acrylamide, (p-N,N-di-n-propylaminophenyl)methyl (meth)acrylamide, (p-N,N-di-n-butylaminophenyl)methyl (meth)acrylamide, (p-N-laurylaminophenyl)methyl (meth)acrylamide, and (p-N-stearylaminophenyl)methyl (meth)acrylamide.

The vinyl monomer having a fluorine-substituted hydrocarbon group is not particularly limited as long as it is used for producing a fluorine-containing resin. Specific examples of the vinyl monomer having a fluorine-substituted hydrocarbon group are fluoroalkyl(meth)acrylates such as 2,2,2-trifluoroethyl acrylate, 2,2,3,3-tetrafluoropropyl acrylate, 2,2,3,3,4,4,5,5-octafluoroamyl acrylate, and 1H,1H,2H,2H-heptadecafluorodecyl acrylate; and fluoroolefins such as trifluorochloroethylene, vinylidene fluoride, trifluoroethylene, tetrafluoroethylene, trifluoropropylene, and hexafluoropropene. Among these, fluoroalkyl(meth)acrylates are preferable.

The addition polymerization process of the monomer having an unsaturated bond may be optionally selected from the processes of solution polymerization, bulk polymerization, emulsion polymerization, and suspension polymerization. Among these production processes, an emulsion polymerization process is preferable since resin fine particles with a uniform particle diameter may be easily obtained.

In the polymerization of the vinyl monomers described above, conventional polymerization initiators such as potassium persulfate, acetyl peroxide, decanoyl peroxide, lauroyl peroxide, benzoyl peroxide, azobisisobutyronitrile, 2,2'-azobis-2,4-dimethyl valeronitrile, and 2,2'-azobis-4-methoxy-2,4-dimethyl valeronitrile may be used. The amount of these polymerization initiators used is preferably from 0.1% to 15% by mass based on the total mass of monomers.

The process for producing the resin fine particles by the emulsion polymerization process is preferably a soap-free emulsion polymerization process using no emulsifying agent (surfactant). In the soap-free emulsion polymerization process, a radical of the initiator occurring in an aqueous phase induces the polymerization of a monomer slightly dissolved in the aqueous phase. As the polymerization progresses, particle cores of insolubilized resin fine particles are formed. The use of the soap-free emulsion polymerization process may result in resin fine particles with a narrow distribution of particle diameters and thus the average particle diameter of the resin fine particles may be easily controlled within a range from 0.03  $\mu\text{m}$  to 1  $\mu\text{m}$ . Therefore, the use of the soap-free emulsion polymerization process may result in the resin fine particles with a uniform particle diameter.

By use of the resin fine particles with a uniform particle diameter obtained through the soap-free emulsion polymerization process, variation of adhesion forces of the resin fine particles to the toner core particles can be reduced and thus a homogeneous shell layer with a uniform thickness can be formed. The resin fine particles produced by the soap-free emulsion polymerization process are formed using no emulsifying agent (surfactant). Therefore, a shell layer resistant to being affected by moisture can be formed by using the resin fine particles obtained through the soap-free emulsion polymerization process.

The resin fine particles may contain components such as a colorant and a charge control agent as described above as required. In cases where the resin fine particles contain a sufficient amount of a charge control agent, the toner core particles may include no charge control agent.

The glass transition point of the resin constituting the resin fine particles is preferably from 45° C. to 90° C. and more preferably from 50° C. to 80° C.

The softening point of the resin constituting the resin fine particles is preferably from 100° C. to 250° C. and more preferably from 110° C. to 240° C. The softening point of the resin constituting the resin fine particles is preferably higher than the softening point of the binder resin in the toner core particles and more preferably 10° C. to 140° C. higher than the softening point of the binder resin. When the shell layer is formed using the resin fine particles consisting of the resin with the softening point within this range, the parts of the resin fine particles contacting the toner core particles are unlikely to deform when the resin fine particles are embedded into the toner core particles. Consequently, convex parts derived from the shape of the resin fine particles prior to forming a shell layer are likely to be formed at an inner surface of the shell layer.

The mass average molecular mass (Mw) of the resin constituting the resin fine particles is preferably from 20,000 to 1,500,000. The mass average molecular mass (Mw) of the resin constituting the resin fine particles can be determined using gel permeation chromatography (GPC) from a molecular mass distribution on a mass basis.

The average particle diameter of the resin fine particles is preferably from 30 nm to 1000 nm, more preferably from 40 nm to 700 nm, particularly preferably from 45 nm to 500 nm, and most preferably from 45 nm to 300 nm. When producing a toner using the resin fine particles with such a particle diameter, the surface of the toner core particles may be easily coated uniformly with the resin fine particles aligned into a monolayer and thus a shell layer with an intended structure may be easily formed.

In cases of producing a toner using the resin fine particles with an excessively small average particle diameter, a shell layer with a preferable thickness may not be formed on the surface of the toner core particles and thus a toner with excellent heat-resistant storage stability may not be obtained. In cases of producing a toner using the resin fine particles with an excessively large average particle diameter, it is difficult to attach the resin fine particles uniformly onto the surface of the toner core particles. Therefore, it is difficult to form the shell layer with a predetermined structure and thus a toner with excellent heat-resistant storage stability is unlikely to be obtained.

The average particle diameter of the resin fine particles can be adjusted by controlling polymerization conditions and using conventional processes such as pulverizing processes and classifying processes. The average particle diameter of the resin fine particles can be computed as a number average particle diameter by measuring a particle diameter for at least 50 resin fine particles from an electron microscope photograph taken using a field emission scanning electron microscope (e.g., JSM-7600F, by JEOL Ltd.).

The amount of resin fine particles used for completely coating the toner core particles can be approximated from an average particle diameter and a specific gravity of toner core particles and an average particle diameter and a specific gravity of resin fine particles. The amount of the resin fine particles used is preferably from 4 to 20 parts by mass and more preferably from 6 to 15 parts by mass based on 100 parts by mass of the toner core particles. When the amount of the resin fine particles used for producing the toner particles is within this range, each of  $D_4$  to  $D_7$  may be easily adjusted to no less than 0.960 and  $(D_{max} - D_{min})$  may be easily adjusted to no greater than 0.015.

In cases where the amount of the resin fine particles used for producing the toner particles is excessively small, the entire surfaces of the toner core particles may not be coated with the resin fine particles. Consequently, sites not covered

with the shell layers may emerge on the surfaces of resulting toner particles. In this case, the resulting toner may be poor in heat-resistant storage stability such as easily agglomerating during storage at high temperatures. Furthermore, the sites not covered with the shell layers emerging on the surfaces of toner particles bring about fine unevenness on the surfaces of toner particles. Consequently, circularity among the average circularities  $D_4$  to  $D_7$  is likely to become less than 0.960 due to the fine unevenness on the surfaces of toner particles. If circularity among the average circularities  $D_4$  to  $D_7$  is less than 0.960, variation tends to appear in the circularities of toner particles. In this case, image defects due to void tend to occur in the images formed using the toner. In cases where the amount of the resin fine particles used is excessively large when producing the toner particles, the shell layer may become thick. In this case, the toner with excellent fixability may not be obtained.

#### External Additive

The toner core particles coated with the shell layer may be treated using an external additive as required. Hereinafter, the particles treated using the external additive is also described as "toner base particles".

The external additive may be exemplified by silica and metal oxides such as alumina, titanium oxide, magnesium oxide, zinc oxide, strontium titanate, and barium titanate. These external additives may be used in a combination of two or more.

The particle diameter of the external additive is preferably from 0.01  $\mu\text{m}$  to 1.0  $\mu\text{m}$ .

The amount of the external additive used is preferably from 0.1% to 10% by mass and more preferably from 0.2% to 5% by mass based on the total mass of the toner base particles produced by forming the shell layer on the surface of the toner core particles. Toner particles treated with an excessively small amount of the external additive exhibits low hydrophobicity. Such a toner which includes toner particles with low hydrophobicity is likely to be affected by water molecules in air under high temperature and high humidity environments. In cases of using a toner, which includes toner particles treated with an excessively small amount of the external additive, problems such as decrease of image density of resulting images due to extreme lowering of the charged amount of the toner and lowering of flowability of the toner tend to occur. In cases of using a toner, which includes toner particles treated with an excessively large amount of the external additive, decrease of image density of resulting images may be caused due to an excessive charge up of the toner particles.

#### Carrier

The toner may be mixed with a desired carrier and used as a two-component developer. In cases of preparing the two-component developer, a magnetic carrier is preferably used as the carrier.

A carrier, whose carrier core material is coated with a resin, may be exemplified as a preferable carrier in cases of using the toner for electrostatic latent image development as the two-component developer. Specific examples of the carrier core material may be exemplified by metal particles such as iron, oxidized iron, reduced iron, magnetite, copper, silicon steel, ferrite, nickel, and cobalt; alloy particles of these materials and metals such as manganese, zinc, and aluminum; alloy particles such as iron-nickel alloy and iron-cobalt alloy; ceramic particles such as titanium oxide, aluminum oxide, copper oxide, magnesium oxide, lead oxide, zirconium oxide, silicon carbide, magnesium titanate, barium titanate, lithium titanate, lead titanate, lead zirconate, and lithium niobate; particles of higher permittivity materials such as ammonium

dihydrogen phosphate, potassium dihydrogen phosphate, and Rochelle salts; resin carriers dispersing these magnetic particles into resins.

Specific examples of the resin, which coats the carrier core material, may be exemplified by (meth)acrylic polymers, styrene polymers, styrene-(meth)acrylic copolymers, olefin polymers (polyethylene, chlorinated polyethylene, and polypropylene), polyvinyl chloride, polyvinyl acetate, polycarbonate, cellulose resins, polyester resins, unsaturated polyester resins, polyamide resins, polyurethane resins, epoxy resins, silicone resins, fluorine resins (polytetrafluoroethylene, polychlorotrifluoroethylene, and polyvinylidene fluoride), phenol resins, xylene resins, diallyl phthalate resins, polyacetal resins, and amino resins. These resins may be used in a combination of two or more.

The particle diameter of the carrier, measured using an electron microscope, is preferably from 20  $\mu\text{m}$  to 200  $\mu\text{m}$  and more preferably from 30  $\mu\text{m}$  to 150  $\mu\text{m}$ .

The apparent density of the carrier, which depends on a carrier composition and a surface structure, is preferably from 2,400  $\text{kg/m}^3$  to 3,000  $\text{kg/m}^3$ .

In cases where the toner is used as a two-component developer, the content of the toner is preferably from 1% to 20% by mass and more preferably from 3% to 15% by mass based on the mass of the two-component developer. By adjusting the content of the toner in the two-component developer within this range, images with an appropriate image density may be successively formed, and pollution inside image forming apparatuses and adhesion of the toner to transfer paper may be suppressed because of suppressing scattering of the toner from developing units.

#### Method of Producing Toner Particles

The method of producing the toner particles in the toner of the present disclosure is not particularly limited as long as toner particles where toner core particles are coated with a shell layer of a predetermined structure can be produced. If desired, external treatment to attach an external additive to a surface of toner base particles may be applied using the toner core particles coated with a shell layer as toner base particles. A preferable method of producing the toner particles in the toner of the present disclosure is explained with respect to a method of producing toner core particles, a method of forming a shell layer, and an external addition treatment method in order below.

#### Method of Producing Toner Core Particles

The method of producing toner core particles is not particularly limited as long as optional components such as a colorant, a release agent, a charge control agent, and a magnetic powder can be appropriately dispersed in a binder resin. A specific example of a desirable method of producing the toner core particles may be such that a binder resin and components including a colorant, a release agent, a charge control agent, and a magnetic powder are mixed using a mixer, then the binder resin and the components to be compounded with the binder resin are melted and kneaded using a kneading machine such as a single or twin screw extruder, and the kneaded material after cooling is pulverized and classified. Typically, the average particle diameter of the toner core particles is preferably from 5  $\mu\text{m}$  to 10  $\mu\text{m}$ .

Furthermore, the toner particles in the toner of the present disclosure represent the average circularities  $D_4$  to  $D_7$ , which are each no less than 0.960. It is therefore preferred that the toner core particles are also prepared such that their average circularities  $D_4$  to  $D_7$  are each around 0.960. The method of producing the toner core particles with such average circularities may be exemplified by (i) and (ii) below:

(i) a method of coarsely pulverizing and finely pulverizing a melt-kneaded material of components in toner core particle followed by heat-treating the resulting pulverized material with a predetermined particle diameter, and

(ii) a method of finely pulverizing the melt-kneaded material by divided multiple stages when pulverizing the melt-kneaded material by coarse pulverizing and fine pulverizing.

The above-mentioned method of fine pulverizing by divided multiple stages in the method (ii) refers to a method in which an operation of once collecting a finely pulverized material from a pulverizing device before average particle diameter of toner particles finely pulverized using the pulverizing device comes to an intended particle diameter and an operation of finely pulverizing again the collected finely pulverized material using the pulverizing device are repeated until the particle diameter of finely pulverized material comes to an intended particle diameter. In a case of producing the toner core particles by a production method including the method (ii), the number of stages in the fine pulverizing step, which is not particularly limited, is preferably at least 3 times.

The mechanical pulverizing device used in the fine pulverizing step may be exemplified by Turbo mill (by Freund-Turbo Co.) and Criptron (by Earthtechnica Co.). When performing the fine pulverizing step by the divided multiple stages, different mechanical pulverizing devices may be used in the respective stages.

#### Method of Forming Shell Layer

The shell layer is formed using spherical resin fine particles. More specifically, the shell layer is formed by a method including:

I) a step of making spherical resin fine particles adhere to the surface of the toner core particles so as to not overlap thereon in a direction perpendicular to the surfaces of the toner core particles and forming layers of the resin fine particles that cover the entire surfaces of the toner core particles, and  
II) a step of smoothening the outer surfaces of the layers of the resin fine particles to thereby form shell layers by applying an external force to the outer surfaces of the layers of the resin fine particles and deforming the resin fine particles in the layers of the resin fine particles.

The method of forming the shell layers using the resin fine particles is preferably a method of using a mixing device capable of mixing the toner core particles and the resin fine particles under a dry condition. A specific method thereof may be exemplified by the method that uses a mixing device capable of applying a mechanical external force to the toner core particles, onto the surfaces of which the resin fine particles have adhered, while making the resin fine particles adhere to the surfaces of the toner core particles and thereby form the shell layers on the surfaces of the toner core particles. The mechanical external force may be exemplified by a shear force that is applied to the toner core particles and that is derived from a shear between the toner core particles themselves or a shear occurring between the toner core particles and an inner wall of the mixing device, a rotor, or a stator; and an impulsive force that is applied to the toner core particles and that is derived from collision between the toner core particles themselves or collision between the toner core particles and an inner wall of the mixing device, when the toner core particles rapidly move within a narrow and small space in the mixing device.

A more specific method is explained. Initially, the toner core particles and the resin fine particles are mixed in a mixing device, thereby making the resin fine particles uniformly adhere to the surfaces of the toner core particles so as to not overlap in a direction perpendicular to the surfaces of the toner core particles. When contacting the toner core par-

title with a large particle diameter and the resin fine particle with a small particle diameter, the surface of the toner core particles microscopically assume a planar surface and the surface of the resin fine particle cause a surface-surface contact. Therefore, the resin fine particle tend to easily adhere to the toner core particle. On the other hand, when contacting the resin fine particles themselves, the contact occurs between curved surfaces of two resin fine particles to thereby cause a point-point contact. Therefore, in the step of making the resin fine particle adhere to the toner core particle, even when a resin fine particle is further adhering to the resin fine particle which has adhered to the surface of the toner core particle, the resin fine particle adhering to the resin fine particle is easily detached from the resin fine particle by a mechanical external force by the mixing device which is applied to the toner core particles to which the resin fine particles have adhered. For this reason, in accordance with the method explained below, the toner core particles are coated with the resin fine particles in a way that the resin fine particles do not overlap in a direction perpendicular to the surface of the toner core particles.

When making the resin fine particles adhere to the toner core particles, the above-mentioned mechanical external force is applied to the layers of the resin fine particles at the surfaces of the toner core particles. As a result, the resin fine particles deform while being embedded into the toner core particles by action of the mechanical external force, and thus the outer surfaces of the layers of the resin fine particles covering the entire surfaces of the toner core particles are smoothed and the layers of the resin fine particles transforms into shell layers. When the shell layers are formed, whereby the smoothening progresses at the outer surfaces of the shell layers, boundary surfaces between the resin fine particles remain inside the shell layers. Therefore, cracks in a direction approximately perpendicular to the surface of the toner core particles are formed inside the shell layer formed using the resin fine particles.

In this stage, when the material of the toner core particles has a hardness equivalent or somewhat higher than that of the resin fine particles forming the shell layer, the inner surface of the shell layer (surface of the side of the toner core particles) may be smoothed. On the other hand, when the material of the toner core particles is softer than the material of the resin fine particles forming the shell layer, the parts of the resin fine particles contacting the toner core particles are resistant to deforming when the resin fine particles are embedded into the toner core particles, therefore, convex parts derived from the shape of the resin fine particles prior to transforming into the shell layer are likely to be formed at the inner surface of the shell layer. In this case, the convex part is formed between two cracks in the shell layer.

In the above-mentioned method, when the mechanical external force is weak, the resin fine particles do not deform to an intended level and thus the shell layer with a predetermined shape may not be formed. Although the condition to form the shell layer with a predetermined shape depends on the type of devices used for forming the shell layer, an appropriate condition for forming a predetermined shell layer can be determined with respect to various devices by confirming the structure of shell layers of toner particles obtained through various conditions while changing operation conditions in a stepwise manner such that the mechanical external force applying to toner core particles coated with resin fine particles becomes larger. However, when the mechanical external force is too large, problems may occur such that the resin fine particles excessively deform and thus cracks in a direction approximately perpendicular to the surface of the

## 21

toner core particles are not formed inside the shell layer or the mechanical external force is converted into heat and thus the toner core particles or the resin fine particles melt.

The devices, allowing to coat the toner core particles using the resin fine particles and also to apply a mechanical external force to the toner core particles coated with the resin fine particles, may be exemplified by Hybridizer NHS-1 (by Nara Machinery Co.), Cosmos System (by Kawasaki Heavy Industries, Ltd.), Henschel mixer (by Nippon Coke & Engineering Co.), Multi-Purpose mixer (by Nippon Coke & Engineering Co.), COMPOSI (by Nippon Coke & Engineering Co.), Mechanofusion system (by Hosokawa Micron Co.), Mechanomill (by Okada Seiko Co.), and Nobilta (by Hosokawa Micron Co.).

## External Addition Treatment Method

The method of treating the toner base particles using an external additive is not particularly limited and the toner base particles can be treated in accordance with methods known heretofore. Specifically, treatment conditions are controlled such that particles of the external additive are not embedded into toner base particles, and the treatment using the external additive is performed by a mixer such as Henschel mixer and Nauta mixer.

The toner for electrostatic latent image development of the present disclosure explained above is excellent in fixability and heat-resistant storage stability, and also occurrence of image defects such as void and letter scattering in resulting images can be suppressed. Accordingly, the toner for electrostatic latent image development of the present disclosure may be favorably used for various image forming apparatuses.

## EXAMPLES

The present disclosure is explained more specifically with reference to examples below. In addition, the present disclosure is not limited to the examples.

## Production Example 1

## Production of Polyester Resin

1960 g of propylene oxide adduct of bisphenol A, 780 g of ethylene oxide adduct of bisphenol A, 257 g of dodeceny succinic anhydride, 770 g of terephthalic acid, and 4 g of dibutyltin oxide were introduced into a reaction container. Next, the atmosphere in the reaction container was changed to nitrogen, and the temperature in the reaction container was raised to 235°C. while stirring. Then, after allowing to react at the same temperature for 8 hours, the pressure inside the reaction container was reduced to 8.3 kPa and the reaction was allowed to proceed for 1 hour. Thereafter, the reaction mixture was cooled to 180°C., and trimellitic anhydride was added to the reaction container so that an acid value of the reaction mixture became an intended value. Then, the temperature of the reaction mixture was raised to 210°C. at a rate of 10°C./hr and reaction was allowed to proceed at the same temperature. After completing the reaction, the content in the reaction container was taken out and cooled, thereby obtaining a polyester resin.

## Production Example 2

## Production of Toner Core Particles

89 parts by mass of a binder resin (the polyester resin obtained through Production Example 1), 5 parts by mass of a release agent (polypropylene wax 660P, by Sanyo Chemical

## 22

Industries, Ltd.), 1 part by mass of a charge control agent (P-51, by Orient Chemical Industries Co.), and 5 parts by mass of a colorant (carbon black MA100, by Mitsubishi Chemical Co.) were mixed using a mixer, thereby obtaining a mixture. Next, the mixture was melted and kneaded using a twin screw extruder, thereby obtaining a kneaded material. The kneaded material was coarsely pulverized using a pulverizing device (Rotoplex, by Toakikai Co.), thereby obtaining a coarsely pulverized material. The coarsely pulverized material was finely pulverized using a mechanical pulverizing device (Turbo mill, by Turbo Industries, Co.), thereby obtaining a finely pulverized material. The finely pulverized material was classified using a classifier (Elbow Jet, by Nitetsu Mining Co.), thereby obtaining toner core particles with a volume average particle diameter ( $D_{50}$ ) of 7.0  $\mu\text{m}$ . The volume average particle diameter of the toner core particles was measured using a Coulter Counter Multisizer 3 (by Beckman Coulter Inc.).

## Production Example 3

## Production of Resin Fine Particles

450 mL of distilled water and 0.52 g of dodecyl ammonium chloride were introduced into a 1000 mL reaction container equipped with a stirrer, a thermometer, a cooling pipe, and a nitrogen-introducing device. The temperature inside the reaction container was raised to 80°C. while stirring the content of the reaction container under nitrogen atmosphere. After raising the temperature, 120 g of an aqueous solution of potassium persulfate (polymerization initiator) with a concentration of 1% by mass and 200 g of deionized water were added to the reaction container. Next, a mixture consisting of 15 g of butyl acrylate, 165 g of methyl methacrylate, and 3.6 g of n-octyl mercaptan (chain transfer agent) was added drop-wise to the reaction container over 1.5 hours followed by further allowing to polymerize over 2 hours, thereby obtaining an aqueous dispersion of resin fine particles. The resulting aqueous dispersion of resin fine particles was dried by freeze-drying, thereby obtaining resin fine particles. The number average particle diameter of the resin fine particles was 0.10  $\mu\text{m}$ .

For the purpose of measuring the number average particle diameter of the resin fine particles, initially, a photograph of the resin fine particles at a magnification of 100,000 times was taken using a field emission scanning electron microscope (JSM-6700F, by JEOL Ltd.). The taken electron microscope photograph was further magnified as required and particle diameters of at least 50 resin fine particles were measured using a measuring device such as a scale and a slide gauge. The number average particle diameter of the resin fine particles was calculated from the measured values.

## Example 1, 2, Comparative Example 1, 2, 4 and 5

## Preparation of Toner Base Particles

Using the amounts described in Table 1 of the resin fine particles obtained through Production Example 3 and 100 g of the toner core particles obtained through Production Example 2, the toner core particles were coated with the resin fine particles and shell layers were formed on the surfaces of the toner core particles. A powder treatment device (Multi-Purpose Mixer Model MP, by Nippon Coke & Engineering Co.) was used for the shell-forming treatment. Specifically, the toner core particles and the resin fine particles were

treated under the rotation numbers and the treatment periods described in Table 1, thereby obtaining toner base particles. External Addition Treatment

The resulting toner base particles were treated with titanium oxide (EC-100, by Titan Kogyo, Ltd.) of 2.0% by mass and hydrophobic silica (RA-200H, by Japan Aerosil Co.) of 1.0% by mass based on the mass of the toner base particles. The toner base particles, the titanium oxide, and the hydrophobic silica were stirred and mixed at a rotational circumferential velocity of 30 m/sec for 5 minutes using a Henschel mixer (by Nippon Coke & Engineering Co.), thereby obtaining toner.

### Comparative Example 3

Using 10 g of the resin fine particles obtained through Production Example 3 and 100 g of the toner core particles obtained through Production Example 2, the toner core particles were coated with the resin fine particles and shell layers were formed on the surfaces of the toner core particles. A surface modification device (device for coating fine particles, Model SFP-01, by Powrex Co.) was used for forming the shell layers. Specifically, toner particles in a toner were prepared by the method below. Initially, the toner core particles were circulated at a charge gas temperature of 80° C. in a fluid bed of the surface modification device. 300 g of an aqueous dispersion of the resin fine particles obtained through Production Example 3, the concentration of which had been adjusted to include 10 g of the resin fine particles, was sprayed into the fluid bed of the surface modification device at a spray speed of 5 g/min for 60 minutes, thereby obtaining toner base particles. The resulting toner base particles were subjected to externally addition treated similarly to Example 1, thereby obtaining a toner of Comparative Example 3.

The toner core particles obtained through Production Example 2 were used as toner base particles and subjected to external treatment similarly to Example 1, thereby obtaining the toner of Comparative Example 6.

### Confirmation of Structure of Shell Layer

In accordance with the method below, surfaces of toner particles in the toners of Example 1, 2 and Comparative Examples 1 to 5 were observed using a scanning electron microscope (SEM) and surface conditions of shell layers coating the toner core particles were confirmed. In accordance with the method below, photographs of cross-sections of the toner particles in the toners of Example 1, 2 and Comparative Examples 1 to 5 were taken using a transmission electron microscope (TEM). Using the resulting TEM photographs, surface conditions of shell layers, conditions inside shell layers, and shapes of inner surfaces of shell layers were confirmed. FIG. 2 shows a TEM photograph of a cross-section of the toner particle in the toner of Example 1, FIG. 3 shows a TEM photograph of a cross-section of the toner particle in the toner of Comparative Example 1, and FIG. 4 shows a TEM photograph of a cross-section of the toner particle in the toner of Comparative Example 3. Since shell-forming treatment was not performed in Comparative Example 6, the toner particles in the toner of Comparative Example 6 was not subjected to SEM observation at a surface of toner particles or TEM observation at cross-sections of toner particles in the toner.

### Method of Observing Surfaces of Toner Particles

Surfaces of toner particles were observed using a scanning electron microscope (JSM-6700F, by JEOL Ltd.) at a magnification of 10,000 times.

### Method of Photographing Cross-Sections of Toner Particles

A sample where toner particles of a toner was enclosed and embedded in a resin was prepared. Using a microtome (EM UC6, by Leica Co.), a thin-piece sample of 200 nm thick for observing cross-sections of the toner particles was prepared from the resulting sample. The resulting thin-piece sample was observed using a transmission electron microscope (TEM, JSM-6700F, by JEOL Ltd.) at a magnification of 50,000 times and an image of an optional cross-section of the toner particles were photographed.

In regards to the toner particles in the toner of Example 1 and 2, the structures derived from spherical resin fine particles could not be observed at the surfaces of shell layers with respect to the toner particles having a particle diameter from 6  $\mu$ m to 8  $\mu$ m when observing the surfaces of the toner particles using the scanning electron microscope (SEM). From the TEM photographs of a cross-sections of toner particles in the toner of Example 1 as shown in FIG. 2, it was confirmed that the outer surfaces of the shell layers of the toner particles in the toner of Example 1 are smooth, cracks in a direction approximately perpendicular to the surfaces of the toner core particles exist inside the shell layers of the toner particles in the toner of Example 1, and the shell layers of the toner particles in the toner of Example 1 have convex parts at the sides of the inner surfaces between two cracks. Since the structure of the shell layer of toner particles in the toner of Example 2 was similar to the structures of the shell layers of toner particles in the toner of Example 1 when observing the cross-section of toner particles in the toner of Example 2 using the TEM, no TEM photograph was taken for the cross-section of toner particle in the toner of Example 2.

In regards to the toner particles in the toners of Comparative Examples 1 and 2, it was confirmed that the surfaces of toner core particles were coated with resin fine particles maintaining a spherical particle state with respect to the toner particles having a particle diameter from 6  $\mu$ m to 8  $\mu$ m when observing their surfaces using the SEM. From the TEM photographs of cross-sections of toner particles in the toner of Comparative Example 1 as shown in FIG. 3, it was confirmed for the toner particles in the toner of Comparative Example 1 that the surfaces of toner core particles were coated with resin fine particles maintaining a particle state. Since the structures of the shell layers of the toner particles in the toner of Comparative Example 2 were similar to the structures of the shell layers of the toner particles in the toner of Comparative Example 1 when observing the cross-sections of the toner particles in the toner of Comparative Example 2 using the TEM, no TEM photograph was taken for the cross-section of the toner particle in the toner of Comparative Example 2.

In regards to the toner of Comparative Example 3, the structures derived from spherical resin fine particles could not be observed at the surfaces of the shell layers with respect to the toner particles having a particle diameter from 6  $\mu$ m to 8  $\mu$ m when observing the surface of the toner particles using the SEM. From the TEM photographs of cross-sections of toner particles in the toner of Comparative Example 3 as shown in FIG. 4, it was confirmed that the outer surfaces of the shell layers of the toner particles in the toner of Comparative Example 3 were smooth. However, from the TEM photographs of the cross-sections of the toner particles in the toner of Comparative Example 3, it could be confirmed that cracks in a direction approximately perpendicular to the surfaces of the toner core particles did not exist inside the shell layers of the toner particles in the toner of Comparative Example 3.

When observing the surfaces of the toner particles in the toners of Comparative Examples 4 and 5 using the SEM, it was confirmed that there were portions, not coated with the

shell layers, on a surfaces of toner core particles. Since the surfaces of toner core particles were not completely coated by the shell layers, the cross-sections of toner particles in the toners of Comparative Examples 4 and 5 were not observed using the TEM.

Toner particles in the toners of Examples 1, 2 and Comparative Examples 1 to 6 were measured for the average circularities  $D_a$ ,  $D_4$ ,  $D_5$ ,  $D_6$ , and  $D_7$  in accordance with the method below. From the measured average circularities  $D_4$  to  $D_7$ , the difference ( $D_{max} - D_{min}$ ) between a maximum value  $D_{max}$  among  $D_4$  to  $D_7$  and a minimum value  $D_{min}$  among  $D_4$  to  $D_7$  was determined. Calculated results of the average circularities of the toners of Examples 1, 2 and Comparative Examples 1 to 6 are shown in Table 1.

#### Method of Calculating Average Circularity

Using a Flow Particle Image Analyzer (FPIA-3000, by Sysmex Co.), an average circularity of toner particles was calculated. Under an environment of 23° C. and 60% RH, a circumferential length ( $L_o$ ) of a circle having a projected area the same as that of a particle image and a peripheral length ( $L$ ) of a particle projected image were measured for all of toner particles. Next, circularities were calculated in accordance with the formula below. Using the data of toner particles with an equivalent circle diameter of no less than 3.0  $\mu\text{m}$  and less than 10.0  $\mu\text{m}$ , the average circularities  $D_a$ ,  $D_4$ ,  $D_5$ ,  $D_6$ , and  $D_7$  were calculated as described below.

#### (Formula to Calculate Circularity)

$$\text{Circularity} = L_o/L$$

#### (Average Circularity $D_a$ of Toner Particles with Particle Diameter of No Less than 3 $\mu\text{m}$ and Less than 10 $\mu\text{m}$ )

The sum of circularities of toner particles to be measured with an equivalent circle diameter of no less than 3.0  $\mu\text{m}$  and less than 10.0  $\mu\text{m}$  was divided by the total particle number of toner particles to be measured with an equivalent circle diameter of no less than 3.0  $\mu\text{m}$  and less than 10.0  $\mu\text{m}$ , and the resulting value was defined as the average circularity  $D_a$ .

#### (Average Circularity $D_4$ of Toner Particles with Particle Diameter of No Less than 4 $\mu\text{m}$ and Less than 5 $\mu\text{m}$ )

The sum of circularities of toner particles to be measured with an equivalent circle diameter of no less than 4  $\mu\text{m}$  and less than 5  $\mu\text{m}$  was divided by the total particle number of toner particles to be measured with an equivalent circle diameter of no less than 4  $\mu\text{m}$  and less than 5  $\mu\text{m}$ , and the resulting value was defined as the average circularity  $D_4$ .

#### (Average Circularity $D_5$ of Toner Particles with Particle Diameter of No Less than 5 $\mu\text{m}$ and Less than 6 $\mu\text{m}$ )

The sum of circularities of toner particles to be measured with an equivalent circle diameter of no less than 5  $\mu\text{m}$  and less than 6  $\mu\text{m}$  was divided by the total particle number of toner particles to be measured with an equivalent circle diameter of no less than 5  $\mu\text{m}$  and less than 6  $\mu\text{m}$ , and the resulting value was defined as the average circularity  $D_5$ .

#### (Average Circularity $D_6$ of Toner Particles with Particle Diameter of No Less than 6 $\mu\text{m}$ and Less than 7 $\mu\text{m}$ )

The sum of circularities of toner particles to be measured with an equivalent circle diameter of no less than 6  $\mu\text{m}$  and less than 7  $\mu\text{m}$  was divided by the total particle number of toner particles to be measured with an equivalent circle diameter of no less than 6  $\mu\text{m}$  and less than 7  $\mu\text{m}$ , and the resulting value was defined as the average circularity  $D_6$ .

#### (Average Circularity $D_7$ of Toner Particles with Particle Diameter of No Less than 7 $\mu\text{m}$ and Less than 8 $\mu\text{m}$ )

The sum of circularities of toner particles to be measured with an equivalent circle diameter of no less than 7  $\mu\text{m}$  and less than 8  $\mu\text{m}$  was divided by the total particle number of toner particles to be measured with an equivalent circle diam-

eter of no less than 7  $\mu\text{m}$  and less than 8  $\mu\text{m}$ , and the resulting value was defined as the average circularity  $D_7$ .

#### Evaluation

In accordance with the method below, fixability, heat-resistant storage stability and transfer performance of the toners of Example 1, 2 and Comparative Examples 1 to 6 were evaluated. Evaluation results of the toners are shown in Table 1. A page printer (FS-05016N, by Kyocera Document Solutions Inc.) modified so as to allow temperature control for evaluation was used as an evaluation apparatus for evaluating fixability and transfer performance. Setting a fixing temperature of the evaluation apparatus to 180° C., evaluation images used for evaluating fixability and transfer performance were obtained under an environment of 20° C. and 65% RH. The evaluation apparatus was allowed to stand in a power-off state for 10 minutes and then powered up for use. A two-component developer, obtained in accordance with the method of Production Example 4 described below, was used for evaluating fixability and transfer property.

#### Production Example 4

##### Preparation of Two-Component Developer

A carrier (ferrite carrier, by Powder-Tech Co.) and a toner of 10% by mass based on the mass of the ferrite carrier were mixed using a ball mill (by Kyocera Document Solutions Inc.) for 30 minutes, thereby preparing a two-component developer.

##### Fixability

5 sheets of recording media having a pattern image for evaluation were output successively using the evaluation apparatus; then, a pattern image for evaluation to measure an image density was output. An image density of solid image of the resulting pattern image for evaluation was measured using a GretagMacbeth reflection density meter (RD914, by GretagMacbeth Co.). Then, the pattern image for evaluation was rubbed using a 1 kg weight coated with a fabric. Specifically, the image for evaluation was rubbed by reciprocating the weight 10 times on the pattern image for evaluation in a way that only its own weight was applied thereto. An image density of the pattern image for evaluation after rubbing was measured using the GretagMacbeth reflection density meter (RD914, by GretagMacbeth Co.). A fixation ratio was calculated from the image densities before and after rubbing of the image for evaluation in accordance with the formula shown below. From the calculated fixation ratio, fixability was evaluated on the basis of the criteria below. Evaluation of "good" was determined to be OK. Fixation Ratio (%) = ((image density after rubbing) / (image density before rubbing)) × 100

Good: fixation ratio of no less than 95%;

Neutral: fixation ratio of no less than 90% and less than 95%; and

Bad: fixation ratio of less than 90%.

##### Heat-Resistant Storage Stability

A toner was stored at 50° C. for 100 hours. Next, the toner was screened using a sieve of 140 mesh (opening 105  $\mu\text{m}$ ) placed on a powder tester (by Hosokawa Micron Co.) under a condition of rheostat scale 5 and period 30 seconds in accordance with a manual of the powder tester. After the screening, a mass of the toner remaining on the sieve was measured. From the mass of the toner before the screening and the mass of the toner remaining on the sieve after the screening, an agglomeration degree (%) of the toner was determined in accordance with the formula shown below. From the calculated agglomeration degree, heat-resistant storage stability

was evaluated on the basis of the criteria below. Evaluation of "good" was determined to be OK.  
(Formula for Calculating Agglomeration Degree)

$$\text{Agglomeration Degree (\%)} = \frac{(\text{mass of the toner remaining on the sieve})}{(\text{mass of the toner before the screening})} \times 100$$

Good: agglomeration degree of no greater than 20%;  
Neutral: agglomeration degree of greater than 20% and no greater than 50%; and  
Bad: agglomeration degree of greater than 50%.

Evaluation of Transfer Performance

As for the evaluation of transfer performance, evaluation of presence or absence of a toner adhering to a developing sleeve (evaluation of sleeve adhesion) and evaluation of occurrence

to be OK. Good: no fouling appeared on the developing sleeve, the solid image as well as the 50% halftone image were good, and no void or letter scattering could be confirmed;

Neutral: fouling appeared on the developing sleeve, image deficiencies (unevenness in sleeve layers) occurred in the solid image and the 50% halftone image by a circumference pitch of the developing sleeve, and void and/or letter scattering could be confirmed; and

Bad: fouling appeared on the developing sleeve, image deficiencies (unevenness in sleeve layers) occurred in the solid image and the 50% halftone image by a circumference pitch of the developing sleeve, and void and/or letter scattering could be confirmed; consequently, the image quality was far from practical use.

TABLE 1

|                                                  | Examples |        | Comparative Examples |         |         |         |         |       |
|--------------------------------------------------|----------|--------|----------------------|---------|---------|---------|---------|-------|
|                                                  | 1        | 2      | 1                    | 2       | 3       | 4       | 5       | 6     |
| Amount of resin fine particles(g)                | 10       | 8      | 10                   | 10      | 10      | 5       | 2       | —     |
| Production conditions                            |          |        |                      |         |         |         |         |       |
| Rotation numbers (rpm)                           | 10,000   | 10,000 | 5,000                | 7,500   | —       | 10,000  | 10,000  | —     |
| Treatment period (min)                           | 10       | 10     | 5                    | 10      | —       | 10      | 10      | —     |
| Measurement results of the average circularities |          |        |                      |         |         |         |         |       |
| $D_a$                                            | 0.967    | 0.962  | 0.965                | 0.966   | 0.969   | 0.962   | 0.955   | 0.949 |
| $D_4$                                            | 0.962    | 0.960  | 0.960                | 0.961   | 0.962   | 0.952   | 0.946   | 0.937 |
| $D_5$                                            | 0.963    | 0.962  | 0.962                | 0.962   | 0.964   | 0.959   | 0.959   | 0.945 |
| $D_6$                                            | 0.965    | 0.964  | 0.965                | 0.965   | 0.966   | 0.965   | 0.965   | 0.951 |
| $D_7$                                            | 0.969    | 0.967  | 0.969                | 0.970   | 0.973   | 0.968   | 0.966   | 0.959 |
| $D_{max} - D_{min}$                              | 0.007    | 0.007  | 0.009                | 0.009   | 0.011   | 0.016   | 0.020   | 0.022 |
| Evaluation                                       |          |        |                      |         |         |         |         |       |
| Fixability                                       | Good     | Good   | Good                 | Good    | Neutral | Good    | Good    | Good  |
| Heat-resistant storage stability                 | Good     | Good   | Bad                  | Neutral | Good    | Neutral | Neutral | Bad   |
| Transfer performance                             | Good     | Good   | Good                 | Good    | Good    | Neutral | Neutral | Bad   |

of void and/or letter scattering in resulting images (evaluation of transfer property) were performed.

(Evaluation of Sleeve Adhesion)

Using the evaluation apparatus, an image was continuously formed on 5,000 sheets under a condition of printing speed 16 sheets/min and coverage rate of 5%; then, a pattern image for evaluation was output after printing the 5,000 sheets. A solid image and a 50% halftone image formed in the pattern image for evaluation and a condition of the developing sleeve of the evaluation apparatus were visually observed.

(Evaluation of Transfer Property)

Using the evaluation apparatus, a thin-line image was formed as an initial image. Presence or absence of void and occurrence of letter scattering on the thin-line image were visually observed using a loupe.

From the evaluation results of sleeve adhesion and transfer property, transfer performance was evaluated in accordance with the criteria below. Evaluation of "good" was determined

50 It is understood from Examples 1 and 2 that a toner is excellent in fixability and heat-resistant storage stability and occurrence of image defects in resulting images due to adhesion of the toner to the developing sleeve and image defects such as void and letter scattering in resulting images can be suppressed when: the toner contains toner particles including

55 toner core particle containing at least a binder resin and a shell layer with a predetermined structure coating the entire surface of the toner core particle, average circularities  $D_4$  to  $D_7$  of toner particles for every specific range of particle diameters are each no less than 0.960, and the difference ( $D_{max} - D_{min}$ ) between a maximum value  $D_{max}$  and a minimum value  $D_{min}$  is no greater than 0.015.

60 It is understood from Comparative Examples 1 and 2 that a toner with good heat-resistant storage stability is unlikely to be obtained when the structures derived from spherical resin fine particles are observed at the surfaces of the shell layers coating the toner core particles. The reason can be estimated

## 29

that when the structures derived from spherical resin fine particles are observed at the surfaces of the shell layers, gaps remain between resin fine particles which have been somewhat deformed, thus components such as a release agent in the toner core particles tend to exude onto surfaces of the toner particles.

It was confirmed from SEM observation of the toner particles of the toners of Example 1 and Comparative Examples 1, 2 that as the rotation number of the device for forming the shell layers is increased, smoothness of the resulting surfaces of the shell layers becomes better.

It is understood from Comparative Example 3 that when cracks in a direction approximately perpendicular to the surfaces of the toner core particles are not observed inside the shell layers, fixability of the resulting toner is poor. The reason is estimated that break of the shell layer is unlikely to occur by the pressure applied to the toner particles during fixing the toner on recording media.

It is understood from Comparative Examples 4 to 6 that image deficiencies (unevenness in sleeve layers) and image defects due to the occurrence of void and letter scattering are likely to occur in resulting images when at least one of  $D_4$  to  $D_7$  is less than 0.960 and  $(D_{max} - D_{min})$  is greater than 0.015.

The invention claimed is:

1. A toner for electrostatic latent image development including a plurality of toner particles, each of the plurality of toner particles comprising a toner core particle containing at least a binder resin and a shell layer coating the toner core particle, wherein:

the shell layer comprises spherical resin fine particles adhere to an entire surface of the toner core particle such that the spherical resin fine particles do not overlap in a direction perpendicular to the surface of the toner core particle,

and

the shell layer further comprises cracks on a surface which is contacting toner core particle, the cracks are approximately perpendicular to surface of the toner core particle and originate at phase boundaries of the resin fine particles themselves, and

with respect to average circularities of the plurality of toner particles in the toner for electrostatic latent image development,

## 30

an average circularity of the plurality of toner particles with a particle diameter of no less than 4  $\mu\text{m}$  and less than 5  $\mu\text{m}$  is defined as an average circularity D4,

an average circularity of the plurality of toner particles with a particle diameter of no less than 5  $\mu\text{m}$  and less than 6  $\mu\text{m}$  is defined as an average circularity D5,

an average circularity of the plurality of toner particles with a particle diameter of no less than 6  $\mu\text{m}$  and less than 7  $\mu\text{m}$  is defined as an average circularity D6, and

an average circularity of the plurality of toner particles with a particle diameter of no less than 7  $\mu\text{m}$  and less than 8  $\mu\text{m}$  is defined as an average circularity D7: each of D4-D7 is no less than 0.960, and

the difference  $(D_{max} - D_{min})$  between a maximum value  $D_{max}$  among D4 to D7 and a minimum value  $D_{min}$  among D4 to D7 is no greater than 0.015.

2. The toner for electrostatic latent image development according to claim 1, wherein a thickness of the shell layer is from 0.05  $\mu\text{m}$  to 0.3  $\mu\text{m}$ .

3. The toner for electrostatic latent image development according to claim 1, wherein when a cross-section of each of the plurality of the toner particles are observed using a transmission electron microscope, a convex part, between two of the cracks, of the shell layer is observable on a phase boundary between the toner core particles and the shell layers.

4. The toner for electrostatic latent image development according to claim 1, wherein the shell layer is formed using a method comprising the steps of I) and II) below:

I) a step of making spherical resin fine particles adhere to the surface of the toner core particle so as to not overlap thereon in a direction perpendicular to the surfaces of the toner core particle and forming a layers of the resin fine particles that cover the entire surfaces of the toner core particle, and

II) a step of smoothening the outer surface of the layer of the resin fine particles to thereby form the shell layer by applying an external force to the outer surface of the layer of the resin fine particles and deforming the resin fine particles in the layers of the resin fine particles.

\* \* \* \* \*